

## UNITED STATES PATENT OFFICE

2,616,785

METHOD OF LOWERING THE TENDENCY  
TOWARDS SETTING OF POTASSIUM NI-  
TRATE AND POTASSIUM NITRATE OF  
FREE-FLOWING FORM WITH A REDUCED  
TENDENCY TO SETTINGAlexander Butchart, North Crescent, Ardrossan,  
Scotland, assignor to Imperial Chemical Indus-  
tries Limited, a corporation of Great BritainNo Drawing. Application April 1, 1949, Serial No.  
85,024. In Great Britain December 29, 1948

8 Claims. (Cl. 23—102)

1

The present invention is concerned with a method of lowering the tendency towards setting of potassium nitrate and with providing potassium nitrate of free-flowing form with a reduced tendency to setting, which is particularly suitable for incorporation in blasting explosives or propellant explosives compositions.

The invention is particularly applicable to potassium nitrate in a state of fine subdivision; that is to say, for example, potassium nitrate ground in a mill to a degree of fineness such that it is capable of passing through a 160 or 200 mesh sieve (BSS). The invention can also be applied to finely divided potassium nitrate produced by a crystallisation process capable of passing through e. g. a 30, 60 or 100 mesh sieve (BSS). Naturally coarsely crystalline free-flowing potassium nitrate, as crystallised in commercial manufacturing processes, for example, potassium nitrate capable of passing through a 10 mesh sieve and retained by a 30 mesh sieve, can also beneficially be treated according to the invention, this coarsely crystalline salt, however, is less prone to setting than finely divided potassium nitrate.

This application is related to application Serial No. 85,728, filed April 5, 1949, to Butchart and Whetstone. That application discloses and claims the formation of a free flowing ammonium sulphate by the addition thereto of small amounts of sulphonated aromatic dyestuff which is soluble in a saturated aqueous solution of ammonium sulphate and which in such solution conditions it to produce on crystallization ammonium sulphate in the form of thin fragile crystals which are friable owing to their facial development relative to the cleavage planes.

According to the present invention the method of lowering the tendency towards setting of potassium nitrate comprises treating the potassium nitrate with a dyestuff of sulphonated aromatic character which in solution in a saturated aqueous solution of potassium nitrate conditions said potassium nitrate solution to produce on crystallization potassium nitrate in the form of thin and fragile crystals, possessing [001] crystal habit and being thereby friable owing to their facial development relative to the cleavage planes of the crystals.

2

According to the present invention potassium nitrate which is in non-cohering and free-flowing form contains a dyestuff of sulphonated aromatic character which in solution in a saturated aqueous solution of potassium nitrate conditions said potassium nitrate solution to produce on crystallisation potassium nitrate in the form of thin fragile crystals, friable owing to their facial development relative to the cleavage planes.

The phrase "dyestuff of sulphonated aromatic character" includes soluble salts of an aromatic dyestuff having at least one sulphonic acid group and aromatic dyestuffs having at least one sulphonic acid substituent group per dye molecule.

Particularly suitable dyestuffs which most markedly lower the tendency towards setting of potassium nitrate are:

- 20 1:4 diamino anthraquinone 2-sodium sulphonate.
- 1:4:5:8 tetraimino anthraquinone disulphonic acid (sodium salt).
- 25 Examples of dyestuffs of sulphonated aromatic character which are soluble in saturated potassium nitrate solution but which in lesser degree than the above reduce the setting tendency of potassium nitrate are:
- 30 Edicol Amaranth (Colour Index No. 184)  
Dyes comprising  $\beta$  naphthol 6-sulphonic acid, or  $\beta$  naphthol 3:6-disulphonic acid coupled with diazotized sulphonated aniline or toluidine.
- 35 Azofuchsine G (Colour Index No. 153)  
Fast Red E (Colour Index No. 182)  
Chlorazol Sky Blue (Colour Index No. 518)  
Acid Green M (Colour Index No. 669)  
Solochrome Black (Colour Index No. 170)
- 40 Tartrazine (Colour Index No. 640)

The following dyestuffs exemplify those soluble in water, and at least slightly soluble in saturated potassium nitrate solutions but which even so have only a slight tendency to reduce the setting and also to maintain the free-flowing nature of potassium nitrate:

- 45 Acid Magenta (Colour Index No. 692)
- Acid Bordeaux B (Colour Index No. 88)
- 50 Carmoisine 6RS (Colour Index No. 29)

Carmoisine LS (Colour Index No. 180)  
 Bismarck Brown (Colour Index No. 331)  
 Hydrazine Yellow SO (Colour Index No. 637)  
 Acid Green G (Colour Index No. 666)  
 Erioglaucine Extra (Colour Index No. 671)  
 Acid Violet 4BNS (Colour Index No. 698)  
 1:5 diamino anthraquinone 2-sulphonic acid.

It has been found that the addition of, for example, between 0.01 and 0.10 part of 1:4 diamino anthraquinone 2-sodium sulphonate or 1:4:5:8 tetramino anthraquinone disulphonic acid (sodium salt) to 100 parts of potassium nitrate capable of passing through a 100 mesh screen lessens the tendency of the potassium nitrate towards caking or setting.

The following examples illustrate how potassium nitrate according to the invention can be produced. The parts are parts by weight.

*Example 1*

A saturated aqueous solution at 40° C. of potassium nitrate containing 0.1% of the added dye 1:4 diamino anthraquinone 2-sodium sulphonate on cooling crystallises in the altered habit of hexagonal plate-like crystals of extreme fragility.

*Example 2*

Potassium nitrate (1000 gm.) ground and sieved through a 100 BSS sieve, is mixed with 10 ml. of water containing in solution 1 gm. of 1:4 diamino anthraquinone 2-sodium sulphonate in a hot water jacketed mixing machine such as a Werner-Pfleiderer incorporator, so that the dye is uniformly distributed over the individual particles. Following evaporation of the added water in the incorporator the finely divided potassium nitrate may be stored for long periods without the occurrence of any hard caking. Untreated potassium nitrate of similar grit is found to cake rapidly under similar conditions involving exposure to atmosphere moisture.

*Example 3*

Potassium nitrate is crystallised with rapid cooling and stirring to give small crystals. The crystals are isolated, and in their wet state are treated with .05% of the dye by spraying with a 10% aqueous solution of 1:4 diamino anthraquinone 2-sodium sulphonate and are then passed through a rotary drier so that the dyestuff is uniformly distributed. The dry salt emerging is found to be free from any tendency towards hard setting under normal storage conditions.

*Example 4*

The procedure is the same as for Example 1 except that 1:4:5:8 tetramino anthraquinone disulphonic acid (sodium salt) is used.

*Example 5*

The procedure is the same as for Example 2 except that 1:4:5:8 tetramino anthraquinone disulphonic acid (sodium salt) is used.

*Example 6*

The procedure is the same as for Example 3 except that 1:4:5:8 tetramino anthraquinone disulphonic acid (sodium salt) is used.

*Example 7*

The procedure is the same as for Example 2 except that Amaranth (C. I. No. 184) is used instead of 1:4 diamino anthraquinone 2-sodium

obtained after evaporation of the added water may be stored for long periods without the occurrence of any hard caking as long as moisture uptakes of the order of 0.2% are not exceeded.

*Example 8*

The procedure is the same as for Example 7 except that Tartrazine (C. I. No. 640) is used instead of Amaranth. The finely divided potassium nitrate obtained has the same characteristics as the potassium nitrate of Example 7.

The procedure is the same as for Example 2 except that "Carmoisine LS" (S. I. No. 180) is used instead of Amaranth. The dry crystals produced show a somewhat lessened tendency towards cohering on standing as compared with similar untreated material.

*Example 9*

The procedure is the same as for Example 2 except that "Carmoisine LS" (S. I. No. 180) is used instead of Amaranth. The dry crystals produced show a somewhat lessened tendency towards cohering on standing as compared with similar untreated material.

*Example 10*

The procedure is the same as for Example 9 except that "Acid Violet 4BNS" (C. I. No. 698) is used instead of "Carmoisine LS." The properties of the dry crystals are the same as those of Example 9.

I claim:

1. A free flowing potassium nitrate comprising crystals of potassium nitrate containing per 100 parts of potassium nitrate, from 0.01 to 0.10 parts of at least one sulphonated aromatic dyestuff distributed predominantly on the surface of the crystal which is soluble to at least the aforesaid extent in a saturated aqueous solution of potassium nitrate and conditions such solution to produce on crystallization potassium nitrate in the form of thin, fragile crystals, possessing [001] crystal habit and being thereby friable owing to their facial development relative to the cleavage planes.

2. A free flowing potassium nitrate as recited in claim 1 in which the dyestuff is 1:4 diamino anthraquinone 2-sodium sulphonate.

3. A free flowing potassium nitrate as recited in claim 1 in which the dyestuff is 1:4:5:8 tetramino anthraquinone disulphonic acid.

4. A free flowing potassium nitrate comprising crystals of potassium nitrate containing per 100 parts of potassium nitrate from 0.01 to 0.10 part of at least one sulphonated aromatic dyestuff predominantly distributed on the surface of the said crystals which is soluble to at least the aforesaid extent in a saturated aqueous solution of potassium nitrate and which in such solution conditions said solution to produce on crystallization potassium nitrate in the form of thin friable crystals, possessing [001] crystal habit and being thereby friable owing to their facial development relative to the cleavage planes.

5. A method for the production of free flowing potassium nitrate in crystalline form which comprises effecting crystallization of an aqueous solution of potassium nitrate containing from 0.01 to 0.1 part per 100 parts of potassium nitrate in solution of at least one sulphonated aromatic dyestuff which is soluble to at least the aforesaid extent in a saturated aqueous solution of potassium nitrate and conditions such solution to produce on crystallization potassium nitrate in the form of thin, fragile crystals, possessing [001] crystal habit and being thereby friable owing to their facial development relative to the cleavage planes.

6. A method for the production of free flowing potassium nitrate as recited in claim 5, which

7. A method for the production of free flowing potassium nitrate in crystalline form which comprises effecting crystallization of an aqueous solution of potassium nitrate containing from 0.01 to 0.1 part per 100 parts of potassium nitrate in solution of at least one sulphonated aromatic dyestuff which is soluble to at least the aforesaid extent in a saturated aqueous solution of potassium nitrate and conditions such solution to produce on crystallization potassium nitrate in the form of thin, fragile crystals, possessing [001] crystal habit and being thereby friable owing to their facial development relative to the cleavage planes.

8. A method for the production of free flowing potassium nitrate as recited in claim 5, which

comprises spraying wet potassium nitrate crystals with an aqueous solution of the dyestuff.

7. A method for the production of free flowing potassium nitrate as recited in claim 5 in which the said dyestuff is 1:4 diamino anthraquinone 2-sodium sulphonate.

8. A method for the production of free flowing potassium nitrate as recited in claim 5 in which the said dyestuff is the sodium salt of 1:4:5:8 tetramino anthroquinone disulphonic acid.

ALEXANDER BUTCHART.

## REFERENCES CITED

The following references are of record in the file of this patent:

## UNITED STATES PATENTS

|    | Number    | Name            | Date           |
|----|-----------|-----------------|----------------|
| 5  | 1,056,365 | Raschig         | Mar. 18, 1913  |
|    | 1,550,064 | Ehrlich         | Aug. 18, 1925  |
|    | 2,009,437 | Coolidge et al. | July 30, 1935  |
| 10 | 2,377,670 | Burdett et al.  | June 5, 1945   |
|    | 2,383,763 | Bloch et al.    | Aug. 28, 1945  |
|    | 2,408,059 | Garfield et al. | Sept. 24, 1946 |